

Oct. 13, 1970

H. W. RIMBACH

3,533,827

METHOD FOR PHOSPHOR COATING AND PHOSPHOR-COATED SUBSTRATE

Original Filed March 11, 1963

2 Sheets-Sheet 1

FIG. 1.



FIG. 3.



INVENTOR  
HENRY W. RIMBACH.

BY

*W. D. Palmer*  
ATTORNEY.

Oct. 13, 1970

H. W. RIMBACH

3,533,827

METHOD FOR PHOSPHOR COATING AND PHOSPHOR-COATED SUBSTRATE

Original Filed March 11, 1963

2 Sheets-Sheet 2



INVENTOR  
HENRY W. RIMBACH.

BY

*W. D. Palmer*  
ATTORNEY

3,533,827

## METHOD FOR PHOSPHOR COATING AND PHOSPHOR-COATED SUBSTRATE

Henry W. Rimbach, Cedar Grove, N.J., assignor to Westinghouse Electric Corporation, Pittsburgh, Pa., a corporation of Pennsylvania

Original application Mar. 11, 1963, Ser. No. 264,248, now Patent No. 3,316,109. Divided and this application Mar. 20, 1967, Ser. No. 644,039

Int. Cl. H01k 1/32

U.S. Cl. 117—33.5

13 Claims

## ABSTRACT OF THE DISCLOSURE

Phosphor powder is adhered to a lamp envelope by first applying to the envelope a film of liquid vehicle having finely divided binder suspended therein. The liquid vehicle comprises a low-boiling component and a high-boiling component and immediately after initial application of the vehicle, the low-boiling component evaporates to leave the high-boiling vehicle component as a viscous layer with the binder suspended therein. The phosphor powder is then impinged as a smoke against the remaining vehicle, and the envelope thereafter heated to complete the coating process. The preferred inorganic binder material is a mixture of finely divided boric oxide and aluminum oxide.

This application is a division of copending application Ser. No. 264,248, filed Mar. 11, 1963, now Pat. No. 3,316-30 109, entitled "Coating Composition," and owned by the present assignee.

This invention generally relates to lamps and, more particularly, to a coating composition for phosphor coating a substrate such as a lamp envelope, a method for adhering phosphor to a substrate such as a lamp envelope, and to a phosphor-coated substrate.

Fluorescent lamps and some high-pressure, mercury-vapor (HPMV) lamps are provided with a phosphor coating which is adhered to the interior surface of the lamp envelope. Such phosphor coatings are normally applied by suspending the phosphor powder in a liquid vehicle which contains a small amount of organic binder material, such as ethyl cellulose or nitrocellulose, in order to impart the desired viscosity to the coating composition. This coating composition is flowed over the interior envelope surface, the vehicle volatilized, and the binder thereafter broken down and removed by heating the coated envelope to a temperature of approximately 650° for about three minutes. This last heating or lehring also serves to adhere the phosphor to the lamp envelope.

In the case of fluorescent lamps, the phosphor is normally coated onto the inner envelope surface so that the phosphor is exposed directly to the discharge plasma. In the case of HPMV lamps, such as described in U.S. Pat. No. 2,748,303, the phosphor is normally coated onto the inner surface of an envelope which surrounds the arc tube, and the phosphor is excited to fluorescence by the generated ultraviolet radiations which pass the arc tube.

Some phosphors are known to be sensitive to the lehring temperatures required to volatilize the organic binder. This decreases the fluorescent brightness of the phosphor. Phosphors which are particularly sensitive to such lehring are those which are activated by stannous tin or cuprous copper or mixtures thereof, and an example of such a phosphor is strontium-magnesium orthophosphate activated by stannous tin. Manganese-activated magnesium fluorogermanate is often used with HPMV lamps, and is not known to be sensitive to lehring temperatures. However, the output of an HPMV lamp incorporating this phosphor is normally about 2½ to 3% lower than that of a clear or uncoated lamp, with only the color of the lamp

and the color rendition of objects illuminated thereby being substantially improved.

It is the general object of the invention to provide a coating composition for adhering phosphor powder to a surface, which coating composition enables the phosphor to be coated without the use of the usual high lehring temperatures.

It is another object to provide a method for adhering phosphor powder to a surface whereby high lehring temperatures are avoided.

It is a further object to provide a phosphor-coated substrate in which the phosphor is adhered to the substrate by means of a selected inorganic binder, which binder causes the performance of the phosphor to be improved.

The aforesaid objects of the invention, and other objects which will become apparent as the description proceeds, are achieved by forming on the substrate which is to be coated, a film of selected liquid vehicle having inorganic binder material suspended therein. A portion of the liquid vehicle is volatilized from the applied film to leave a viscous, non-flowing residue of binder and vehicle. Against this still-wet film is impinged a phosphor powder. The residual portion of the liquid vehicle wets the phosphor powder and causes it to adhere to the surface being coated. Thereafter, the remaining liquid vehicle is volatilized from the film. There is also provided a coating composition for adhering phosphor to a surface, which coating composition comprises a mixture of liquids having varying vapor pressures, with the finely divided inorganic binder material suspended therein. There is additionally provided a phosphor-coated substrate, wherein a particular binder material is used in order to cause the coated phosphor to have improved performance characteristics.

For a better understanding of the invention, reference should be had to the accompanying drawings, wherein:

FIG. 1 is an elevational view, partly in section, illustrating an HPMV lamp wherein the inner surface of the outer envelope carries a coating of phosphor material applied in accordance with the present invention;

FIG. 2 is an elevational view, partly in section, illustrating the phosphor coating step wherein a smoke of phosphor powder is being impinged against a bulb which has previously been coated with the coating composition of the present invention; and

FIG. 3 is a flow chart which sets forth the steps of the present method.

With specific reference to the form of the invention illustrated in the drawings, in FIG. 1 is shown an HPMV lamp 10 which has an exterior envelope 12 coated with phosphor in accordance with the present invention. The lamp 10 generally corresponds to the lamp as described in the aforesaid Pat. 2,748,303, which patent may be referred to for details. Briefly, the exterior envelope 12 surrounds a quartz arc tube 14 which is coaxially disposed therein. The arc tube 14 is held by a suitable supporting frame 16 which also serves as one electrical connection. Operating electrodes 18 are disposed in the opposite ends of the arc tube 14. A starting electrode 20 is disposed at one end of the arc tube 14, and is electrically connected to the supporting frame 16 through a suitable starting resistor 22. The lead-in conductors 24 are sealed through the neck of the outer envelope 12 by means of a conventional re-entrant stem 26 and electrical connection is facilitated by a conventional screw-type base 28.

The coating composition which is used to adhere the phosphor to the interior envelope surface comprises a liquid vehicle which has a predetermined amount of selected, inorganic binder material suspended therein. The liquid vehicle of the coating composition comprises a mixture of a first liquid having a relatively high vapor pressure at normal room temperature and other liquid which has a relatively low vapor pressure at normal

room temperature. These liquids are mixed in miscible proportions and are capable of wetting the surface to be coated. The binder material, which is suspended in finely divided form throughout the liquid vehicle, is chosen so that when substantially dry and positioned in contacting relationship between the phosphor and the surface to be coated, it will bind the phosphor to the surface. To avoid discoloration, the liquid vehicle and binder are so chosen as to be substantially chemically inert with respect to one another, although a small proportion of the total binder material may be dissolved in the liquid vehicle.

The relative proportions of the low-vapor-pressure liquid and the binder suspended therein are such that when these two ingredients are mixed together, without the presence of the liquid which has a relatively high vapor pressure, the mixture has sufficient viscosity to substantially prevent free flow when coated as a thin film on the surface which is to be phosphor coated. The viscosity of the low-vapor-pressure liquid and suspended binder is too great, however, to permit such a mixture to be coated as a substantially uniform thin film over the surface which is to be phosphor coated. To permit easy application of the coating composition, it is necessary to include as a part of the coating composition a predetermined proportion of the liquid which has a relatively high vapor pressure. This composite coating composition has a sufficiently low viscosity to permit same to be coated and flow over the surface as an adherent thin film.

The coating composition may be applied to the surface to be phosphor coated in any conventional manner, such as flowing or spraying, although it has been found advantageous merely to flow the coating composition over the surface to be coated, such as an open-necked bulb 30, as shown in FIG. 2. Immediately after a film of the coating composition has been applied to the interior surface of the bulb 30, the high-vapor-pressure liquid vehicle portion thereof volatilizes, leaving as a residue an adherent, non-flowing, thin film of the low-vapor-pressure liquid which has the finely divided inorganic binder material suspended therein.

After at least a substantial portion of the high-vapor-pressure (low boiling) liquid constituent of the coating composition has been volatilized, a smoke of phosphor powder is impinged against this still-wet but very viscous residual film which adheres to the envelope surface. Preferably a phosphor smoke is created by forcing compressed air through a reservoir 32, which contains a supply 34 of the phosphor to be coated. The phosphor is carried as a smoke from the reservoir 32, through an elongated conduit 36, and is impinged against a target 38, which causes the phosphor to disperse as a smoke cloud. During this coating operation, the bulb 30 is retained at its dome portion by a conventional friction clamp 39, which is adapted to be rotated during phosphor coating by a conventional motor-gear arrangement 40. In the coating operation as shown, the elongated feed conduit 36 is gradually introduced into the rotating bulb 30, in order to uniformly coat the desired amount of phosphor onto the still-wet interior surface of the bulb 30. After the phosphor is completely coated, the residual low-vapor-pressure liquid which remains on the interior surface of the bulb is volatilized, either by heating or allowing the bulb to stand for a relatively prolonged period. This causes the inorganic binder material to contact both the phosphor and interior bulb surface, which in turn adheres the phosphor to the bulb 30. The essential steps of the method for applying the phosphor are shown in the flow diagram of FIG. 3.

As a specific example, the liquid vehicle component of the present coating composition which has a relatively low vapor pressure (and a high boiling point) is ethylene glycol monobutyl ether acetate, and the component of the liquid vehicle which has a relatively high vapor pressure is methanol. In the case of this acetate-methanol liquid vehicle, the methanol desirably comprises from 80% to

70% by weight of the total liquid in the coating composition, and the acetate comprises from 20% to 30% by weight of the total liquid in the coating composition. Other suitable high-boiling organic liquids which have a relatively low-vapor-pressure can be substituted for the foregoing preferred example, such as diethylene glycol monoethylether acetate. Other low-boiling liquids which have a relatively high vapor pressure can be substituted for the preferred methanol, and an example is ethanol.

It has been found that the vapor pressure of the high-boiling component of the liquid vehicle desirably is from 0.005 mm. to 2 mm. Hg at normal room temperature, with the preferred vapor pressure for this component being from 0.01 mm. to 0.05 mm. Hg at normal room temperature. The vapor pressure for the low-boiling component of the liquid vehicle desirably is from 200 mm. to 17 mm. Hg at normal room temperature, with the preferred vapor pressure for this component being from 200 mm. to 30 mm. Hg at normal room temperature. As a specific example, the methanol and ethylene glycol monobutylether acetate are present in the liquid vehicle component of the composition in the ratio by weight of 76%-24%.

The preferred finely divided, inorganic binder material is alumina, such as is available under the trademark "Alon C." In order to obtain best results with respect to improved phosphor performance, however, it is desirable to use an inorganic binder which comprises a mixture of the indicated alumina as well as boric oxide. Of course when the composition is initially applied, the boric oxide in all probability is present in large part as boric acid, but when the lamp is baked during final exhaust, substantially all water present in the boric oxide and alumina is removed. Since the degree of hydrolysis of the boric oxide in the coating composition can vary, the weight percentages of this coating composition component are expressed in terms of the oxide, rather than the acid. Desirably the total binder in the coating composition is present in amount of from 1.5 grams to 23.5 grams per 100 cc. of total liquid in the coating composition, with the alumina present in an amount of from 1.5 grams to 15 grams per 100 cc. and the boric oxide present in amount of up to 8.5 grams per 100 cc. The preferred range for binder materials is from 6.5 grams to 10.5 grams alumina and from 2.5 grams to 5 grams of boric oxide per 100 cc. of total liquid. As a specific example, a binder combination of about 8.5 grams of alumina and about 3.4 grams of boric oxide per 100 cc. of total liquid has been found to give very good results.

As a detailed specific example, 50 cc. of methanol are mixed with 16 cc. of ethylene glycol monobutyl ether acetate, along with 5.6 grams of the finely divided alumina and 2.2 grams of boric oxide. This coating composition is flowed over the envelope surface to leave a uniform film approximately 46 microns thick. The methanol volatilizes almost immediately, leaving a substantially uniform film having a thickness of about 11 microns. The amount of finely divided binder material is such that the binder and liquid acetate form a very viscous "slush" which will not flow readily under the forces of gravity.

Thereafter the phosphor smoke is impinged against the still-wet coating "slush." Because of the viscosity of the remaining coating and the relatively large size of the phosphor particles, a substantial portion of the phosphor is only partially immersed into the remaining coating composition. The amount of the phosphor which is utilized is not particularly critical, but desirably is from 1 to 20 milligrams of phosphor per square centimeter of surface area being coated, and preferably is from 2 to 10 milligrams of phosphor per square centimeter of surface area being coated. The remaining liquid vehicle portion of the formed film of the coating composition is then volatilized, preferably by heating the phosphor-coated bulb to a temperature of about 300° C. for a period of about 20 minutes. Thereafter the lamp fabrication is completed in accordance with conventional procedures. The coarser phosphor par-

ticles have shown better performance characteristics, particularly in the case of either copper-activated phosphors, such as disclosed in U.S. Pat. No. 3,025,423, or tin-activated strontium-magnesium orthophosphate.

In tests on a large number of lamps coated in accordance with the present method, the initial light output, as well as the maintenance of light emission for HPMV lamps utilizing cuprous-copper-activated or stannous-tin-activated phosphors is greatly improved. In the case of a strontium-magnesium phosphate activated by stannous tin, the initial light output is greater than the control lamps by about 2000 lumens. After 2500 hours operation, 400 watt HPMV lamps utilizing the strontium-magnesium phosphate phosphor, coated in accordance with the present invention, display an output which is about 2000 lumens greater than that of the control lamps. Some but not all of this improvement can be attributed to the fact that this particular phosphor is sensitive to usual lehring temperatures as required to volatilize organic binder, which lehring is not used when coating in accordance with the present method.

A most unexpected improvement has been found in the case of the fluorogermanate phosphor, which phosphor has been considered as relatively insensitive to high lehring temperatures. 400 watt HPMV lamps coated as per the present invention with magnesium fluorogermanate phosphor display an initial (100 hour) output approximately 1150 lumens greater than otherwise similar factory control lamps which were phosphor coated using organic binder and then lehred. After 500 hours operation, these same lamps displayed an output which averaged 1500 lumens greater than the phosphor-coated factory control lamps. The mechanism by which this improved performance is obtained is not understood, since it has always been assumed that the total output of a fluorogermanate-coated HPMV lamp could not be substantially improved over that of a clear lamp. Whatever the explanation, the foregoing improved results have been consistently achieved.

While the foregoing description considers in detail a phosphor-coated HPMV lamp, it should be understood that the present coating procedures can also be used to coat fluorescent tubes with phosphor, such as the well-known halophosphates. One advantage of such a coating procedure is the elimination of the very high lehring temperatures required to burn out the organic binder, thereby minimizing impurities which may be driven from the glass, and also eliminating the possibility that all of the organic binder material is not volatilized during lehring.

It will be recognized that the objects of the invention have been achieved by providing an improved method for adhering phosphor powder to a substrate, a coating composition which enables a phosphor material to be adhered to a substrate without lehring at high temperatures, and an improved phosphor coating, wherein the coated phosphor has improved performance characteristics.

While best examples of the invention have been illustrated and described in detail, it is to be particularly understood that the invention is not limited thereto or thereby.

I claim as my invention:

1. The method of adhering finely divided phosphor to a surface of a glass envelope, which method comprises:
  - (A) applying as a film to said surface, a predetermined amount of coating composition comprising:
    - (a) a liquid vehicle comprising a mixture of first liquid having a relatively high vapor pressure at normal room temperature and other liquid having a relatively low vapor pressure at normal room temperature, said liquids mixed in predetermined miscible proportions and capable of wetting said surface;
    - (b) a predetermined amount of selected inorganic binder material at least a substantial proportion of which is suspended in finely divided form throughout said liquid vehicle, said liquid vehicle

and said binder being substantially chemically inert with respect to one another, and said binder when substantially dry and positioned intermediate and in contacting relationship with said phosphor and said surface binding said phosphor to said surface;

- (c) the relative proportions of said low-vapor-pressure liquid and said binder being such that when mixed together without said first liquid, the mixture has sufficient viscosity to substantially prevent free flow when coated as a film on said surface; and
  - (d) said composition having a sufficiently low viscosity to permit said composition to be coated and flow over said surface as an adherent film;
- (B) volatilizing at least a portion of said first liquid from said applied film to leave a non-flowing viscous residue adherent to said surface;
- (C) impinging against said viscous residue, a smoke of said phosphor to adhere said phosphor to said surface by means of residual liquid remaining in said film; and
- (D) volatilizing remaining liquid from said film to cause said inorganic binder to bind said phosphor to said surface.

2. The method as specified in claim 1, wherein the amount of finely divided phosphor impinged against said surface is from about 1 to 20 mg. per sq. cm. of surface area being coated.

3. The method as specified in claim 1, wherein the amount of finely divided phosphor impinged against said surface is from about 2 to 10 mg. per sq. cm. of surface area being coated.

4. The method as specified in claim 3, wherein said first liquid has a vapor pressure of from 200 torrs to 17 torrs at normal room temperature, and said second liquid has a vapor pressure of from 0.005 torr to 2 torrs at normal room temperature.

5. The method as specified in claim 4, wherein said first liquid is methanol, and said second liquid is ethylene glycol monobutyl ether acetate, with said methanol constituting from 80% to 70% by weight of the total liquid and said acetate constituting from 20% to 30% by weight of the total liquid.

6. The method as specified in claim 5, wherein said binder is present in total amount of from 1.5 grams to 23.5 grams per 100 cc. of said liquid vehicle, said binder consists of aluminum oxide with or without additional boric oxide, said aluminum oxide is present in amount of from 1.5 grams to 15 grams per 100 cc. of said liquid vehicle, and said boric oxide is present in amount of up to 8.5 grams per 100 cc. of said liquid vehicle.

7. The method as specified in claim 6, wherein said liquid acetate portion of the formed film is volatilized by heating to a temperature of about 300° C.

8. The method of adhering finely divided phosphor to the interior surface of a glass envelope, which method consists of:

- (A) applying as a film to said surface a predetermined amount of coating composition consisting of:
  - (a) a liquid vehicle consisting of a mixture of methanol and ethylene glycol monobutyl ether acetate mixed in proportions of from 80% to 70% by weight methanol and from 20% to 30% by weight acetate;
  - (b) from 9 grams to 15.5 grams per 100 cc. of said liquid vehicle of a binder consisting of a mixture of finely divided aluminum oxide and boric oxide, with the alumina constituting from 6.5 to 10.5 grams per 100 cc. of said liquid vehicle and the boric oxide constituting from 2.5 to 5 grams per 100 cc. of said liquid vehicle;
- (B) volatilizing at least a portion of said methanol from said applied film to leave a non-flowing viscous residue adherent to said surface;

- (C) blowing and impinging against said viscous residue, a smoke of said phosphor to adhere said phosphor to said surface by means of residual liquid remaining in said film; and  
 (D) volatilizing remaining liquid from said film by heating to a temperature of about 300° C. to cause said inorganic binder to bind said phosphor to said surface.  
 9. The method of adhering phosphor as specified in claim 8, wherein said predetermined amount of coating composition is applied as a film to said surface to a thickness of approximately 46 microns.

10. A glass envelope, finely divided phosphor adhered to the interior surface of said envelope by means of an inorganic binder, said binder consisting of a mixture of aluminum oxide and boric oxide, aluminum oxide in said binder present in amount of from 0.07 to 0.7 mg./cm.<sup>2</sup> of surface area of coated envelope, and boric oxide in said binder present in amount of from 0.03 to 0.42 mg./cm.<sup>2</sup> of surface area of coated envelope, and said phosphor present in amount of from 1 to 20 mg./cm.<sup>2</sup> of surface area of said coated envelope.

11. A glass substrate, finely divided phosphor adhered to a surface of said substrate by means of inorganic binder, said binder consisting essentially of a mixture of aluminum oxide and boric oxide, aluminum oxide in said binder present in amount of from 0.07 to 0.7 mg./cm.<sup>2</sup> of surface area of coated substrate, and boric oxide in said binder present in amount of from 0.03 to 0.42 mg./cm.<sup>2</sup> of surface area of coated substrate.

12. A glass substrate, finely divided phosphor adhered to a surface of said substrate by means of inorganic binder,

said binder consisting essentially of a mixture of aluminum oxide and boric oxide, aluminum oxide in said binder present in amount of from 0.25 to 0.5 mg./cm.<sup>2</sup> of surface area of coated substrate, and boric oxide in said binder present in amount of from 0.03 to 0.23 mg./cm.<sup>2</sup> of surface area of coated substrate, and said phosphor present in amount of from 2 to 10 mg./cm.<sup>2</sup> of surface area of coated substrate.

13. A glass substrate, finely divided phosphor adhered to a surface of said substrate by means of inorganic binder, said binder consisting essentially of a mixture of aluminum oxide and boric oxide, aluminum oxide in said binder present in amount of about 0.4 mg./cm.<sup>2</sup> of surface area of coated substrate, and boric oxide in said binder present in amount of from 0.05 to 0.11 mg./cm.<sup>2</sup> of surface area of coated substrate, and said phosphor being present in amount of from 2 to 10 mg./cm.<sup>2</sup> of surface area of coated substrate.

#### References Cited

##### UNITED STATES PATENTS

2,527,134 10/1950 Johnson ----- 117—33.5 XR  
 2,660,686 11/1953 Putnam ----- 117—33.5 XR

##### FOREIGN PATENTS

25 963,638 10/1960 Great Britain.

ALFRED L. LEAVITT, Primary Examiner

W. F. CYRON, Assistant Examiner

30 U.S. CL. X.R.

117—106